

# United States Patent [19]

Fumei

[11] Patent Number: 4,612,721

[45] Date of Patent: \* Sep. 23, 1986

- [54] **CONTAINER WITH SOLID PLASTIC LABEL AND METHOD OF APPLYING THE LABEL**

[75] Inventor: **Giancarlo J. Fumei, Perrysburg, Ohio**

[73] Assignee: **Owens-Illinois, Inc., Toledo, Ohio**

[\*] Notice: The portion of the term of this patent subsequent to Feb. 4, 2003 has been disclaimed.

[21] Appl. No.: **555,787**

[22] Filed: **Nov. 28, 1983**

[51] Int. Cl.<sup>4</sup> ..... **G09F 3/00**

[52] U.S. Cl. ..... **40/310; 40/2 R;**  
..... **40/21 R; 40/306**

[58] Field of Search ..... **40/306, 310, 625, 2 R;**  
..... **156/455**

### References Cited

## U.S. PATENT DOCUMENTS

- |           |         |                       |         |
|-----------|---------|-----------------------|---------|
| 2,002,900 | 5/1935  | Leibig .....          | 40/310  |
| 2,984,596 | 5/1961  | Franer .....          | 40/630  |
| 3,235,433 | 2/1966  | Cvacho et al. ....    | 156/229 |
| 3,472,722 | 10/1969 | Hutchinson .....      | 156/455 |
| 3,542,229 | 11/1970 | Beyerlein et al. .... | 40/310  |
| 3,599,362 | 8/1971  | Klober .....          | 40/310  |
| 3,604,584 | 9/1971  | Shank .....           | 40/310  |
| 3,657,043 | 4/1972  | Ploetz .....          | 40/310  |

- |           |        |                    |        |
|-----------|--------|--------------------|--------|
| 4,004,705 | 1/1977 | Fujio .....        | 40/310 |
| 4,024,009 | 5/1977 | Amsden et al. .... | 40/310 |
| 4,273,816 | 6/1981 | Tollette .....     | 40/615 |
| 4,324,058 | 4/1982 | Sherwick .....     | 40/310 |
| 4,465,717 | 8/1984 | Crofts et al. .... | 40/2 R |

*Primary Examiner*—Gene Mancene

*Assistant Examiner*—Wenceslao J. Contreras

*Attorney, Agent, or Firm*—John R. Nelson

[57] ABSTRACT

The present invention provides, without the drawbacks accompanied by the use of hot melt adhesives, an attractive, easily recycled labelled container, the solid polymer label, on its underside that is adjacent the container when applied, being provided with a finite area on its leading edge and a finite area on its trailing edge, by applying thereto a solvent for the polymer in each of the finite areas, the finite areas comprising a viscous tacky solution of the polymer in the solvent, the solidifying solution being sufficient to tack and bond the label to container during wrapping.

After the label is wrapped around the container, the bond between the container and label becomes weaker as the solidifying solution hardens so that later the label can be easily and cleanly stripped from the container for recycling.

## 16 Claims, 6 Drawing Figures





FIG. 4



FIG. 2



FIG. 3



## CONTAINER WITH SOLID PLASTIC LABEL AND METHOD OF APPLYING THE LABEL

The present invention relates to a container and a plastic label wrapped therearound, and to a method of applying the label to the container.

### BACKGROUND OF THE INVENTION

It has been known to utilize mechanical handling apparatus to supply labels to a container. Such apparatus has included a plastic label sheet feed supply, a drum upon which the label is secured and which moves the label into engagement with the outer surface of a container. The label adheres to the container and is subsequently wrapped around the container by rolling it along a fixed surface. U.S. Pat. No. 4,323,416, for instance, shows such an apparatus, the label being glued to the container and its overlapped ends glued together by the use of a glue applicator assembly. Hot melt adhesives have been used to secure the labels to the container and to form a glued side seam when applied to the overlapped label ends.

Other adhesives, with accompanying drawbacks, have been used such as dextrines and other water-based adhesives, and pressure sensitive adhesives. For containers such as oriented plastic carbonated beverage bottles, pressure sensitive adhesives have not been commonly used.

The use of the hot melt adhesive (glue) has been messy and expensive, heat being required to heat the adhesive. There is a hazard of being exposed to possible burning from heaters used to heat the glue. In addition, such as in the case of an oriented plastic container, the label cannot be easily removed from the container and hence the body portion of the container is contaminated and cannot be readily recycled.

### OBJECTS OF THE INVENTION

It is an object of the present invention to provide apparatus and methods for quickly and efficiently applying plastic labels to a container in a production basis without using a hot melt adhesive with its resultant drawbacks.

It is an object of the present invention to provide an attractive product that is easily recycled, a plastic label being wrapped around a container using a solvent-seal system that eliminates the drawbacks associated with the use of hot melt adhesive systems.

It is an object of the present invention to provide a method of labelling containers and the attractive, easily recycled labelled container itself, the container having a neck and a body, and a plastic label wrapped around the body, the label made of a thermoplastic polymer that is printable and is soluble in a solvent, the label comprising a solid polymer layer having a side that contacts the body and is attached lightly but securely thereto, the foam layer having a leading edge for contacting the body, there being a finite area on the leading edge having a liquid viscous solution of a polymer in a solution in the finite area being adapted to solidify and form a solid bond, the solution forming a momentary tacky bond sufficient to anchor the leading edges to the container body whereby the label can be wrapped around the body, the bond between the label and body becoming weaker as the solidifying solution hardens whereby the label can be easily removed from the container body for recycling without contaminating the material of the

container body being reclaimed, the solid layer having a trailing edge that overlaps the leading edge to form a sleeve label with overlapped edges on the container body, and the solid layer of the trailing edge containing a second finite area generally extending along the trailing edge, the second finite area comprising a liquid tacky solution of a polymer in a solvent, the solution solidifying to form a side seam bond on the overlapped edges, the bond becoming stronger whereby, upon use, the side seam resists being pulled apart.

### DESCRIPTION OF THE DRAWINGS

These and other objects will be apparent from the specification that follows, the appended claims, and the drawings, in which:

FIG. 1 is an elevational view of a container in the form of an oriented plastic container with a base cup;

FIG. 2 is a perspective view of the container of FIG. 1 with a label being partially wrapped around the container;

FIG. 3 is a top plan view of the plastic label shown in FIG. 2, the label having on its underside a plurality of finite areas near its leading edge and a finite area in the form of a strip near its trailing edge, the finite areas formed on the label momentarily before wrapping, the finite areas being a viscous tacky solution of the polymer from the label in a solvent therefor, the solution solidifying to form a solid bond;

FIG. 4 is an enlarged fragmentary sectional view of the plastic label; and

FIGS. 5 and 6 are each top plan views of the plastic label showing different embodiments thereof.

### THE INVENTION

The present invention provides, without the drawbacks accompanied by the use of hot melt adhesive glues, an attractive, easily recycled labelled container, the label, on its underside that is adjacent the container when applied, being provided with a finite area on its leading edge and a finite area on its trailing edge, by applying thereto a solvent for the polymer in each of the finite areas, the finite areas comprising a viscous tacky solution of the polymer in the solvent, the solidifying solution being sufficient to tack and bond the label to container during wrapping.

After the label is wrapped around the container, the bond between the container and label becomes weaker as the solidifying solution hardens so that later, the label can be easily and cleanly stripped from the container for recycling.

As used herein, the term solidification refers to a process resulting from solvent evaporation from an applied area or migration into areas adjoining the area of application. The rate of solidification is due to the rate that the above process takes place and is dependent upon the boiling point of the solvent, the amount applied and the solubility of polymer in the solvent.

The present invention also provides a clean and quick method of applying a plastic label comprising a solid polymer layer to a container having a body portion, the method comprising the steps of:

A. positioning the label around the container body by advancing a leading lateral edge, the label having an outer surface with indicia thereon and an under surface disposed adjacent the body portion,

B. contacting the leading edge of the solid polymer layer with a solvent for the polymer,

C. forming a finite area on the polymer leading edge from the contacting with the solvent,

D. tacking the layer to the body portion by placing the finite area with a liquid tacky solution of the polymer in the solvent next to the body portion,

E. solidifying the tacky liquid to form a tacky adhesive bond between the solid layer and the body portion so that the label can be wrapped around the body, the bond becoming weaker as the solidifying solution hardens so that, after use, the label can be easily stripped from the container for recycling,

F. forming a finite area containing a liquid tacky solution of layer polymer in a solvent on the under surface of the trailing edge,

G. overlapping the trailing and leading edges to form a seam; and

H. bonding the edges of the seam together by solidifying the liquid tacky solution to form a solid bond between the upper and under surfaces of the solid plastic layer.

U.S. Pat. No. 3,468,467 to Amberg (assigned to Owens-Illinois, Inc.) shows a two piece plastic cup construction with a solvent seal for the side seam and solvent sealing the bottom in place. The Amberg patent discloses the use of methylene chloride as a solvent for use with the hard, dense polystyrene skin of the cup material. The sealing is performed fairly slowly and the use of pressure on the overlapped edges of the side seam, etc. is disclosed. The text of the Amberg patent contains in several places a prohibition against the use of the solvent in the foam area of the polystyrene material. For instance, see lines 14-20 in column 2.

In sharp contrast, the present inventor uses a solvent sealing system in which the solvent, methylene chloride, is applied directly to the polystyrene layer of a plastic label. The methylene chloride dissolves the polystyrene in the solid layer. The timing of the solidification of the resultant tacky solution is such that the solid layer can be lightly and securely tacked to the container surface by the solidifying solution within  $\frac{1}{2}$  or preferably within  $\frac{1}{3}$  of a second so it can be wrapped on a production basis. The methylene chloride is also applied to the trailing edge of the polystyrene label to form a finite area on the trailing edge that forms a side seam seal when the label ends are overlapped, the finite area being formed with a solidifying tacky solution of polystyrene in methylene chloride.

As seen in the drawings, a container 8 having a body portion 9 and a base cup 9a is shown partially wrapped with a label 10 in FIG. 3.

As seen in FIGS. 2 and 4, in the embodiment shown, the label has a solid polymer layer 20. The layer 20 has an underside 22, a leading edge 25 and a trailing edge 27. Finite areas 65 are provided on the underside near the leading edge and a finite area 66 is provided on the trailing edge. These finite areas are momentary, solidifying tacky solutions of the polymer in the finite area and the solvent therefor, the preferred solution being one of polystyrene in methylene chloride.

The novel container and label therefor of the present invention is suitable for high production as shown in copending U.S. patent application for an invention of Harold R. Fosnaught, filed the same day as the application, entitled "Apparatus and Method for Wrapping a Plastic Label Around a Container," it being assigned to the same assignee as this application. The disclosure of the above-described application of the apparatus and method for automatically applying plastic labels to con-

ainers using a solvent-seal system on a high volume basis is hereby incorporated by reference.

Polystyrene is a highly preferred polymer for the polymer of the finite area to form the momentary tacky solution on the leading edge so the label can be wrapped on the container. A suitable solid polystyrene layer, which is preferably treated with methylene chloride, has a density of about at least 62 or 63 and preferably 64-65 lbs. per cubic foot.

Other preferred polymers that can be used for part or all of the polystyrene, for most applications, are styrenic polymers such as copolymers of styrene and a vinyl copolymerizable monomer including vinyl acetate, vinyl chloride, vinylidene chloride and acrylic and acrylate monomers such as methyl methacrylate and ethyl methacrylate methyl acrylate and ethyl acrylate. It is preferred that the amount of styrene in styrenic polymer be at least about 40 or 50% by weight and, for best results, about 60 to 75%.

Polymers that can be used in place of polystyrene at least for some applications include polyvinylchloride and acrylate polymers such as polymethyl methacrylate polyethyl methacrylate, polymethylacrylate, polyethylacrylate.

The thickness of the solid layer can vary from about 1 up to about 15 or 20 mils, but the preferred thickness is about 2 to 5.

An outstanding label that has been used is one that is multilayered. The multilayered label can be laminated, but is preferably a coextruded structure of a solid polymer layer such as polystyrene and a solid layer of another styrenic polymer. One of the solid layers of the multilayered label can be about  $\frac{1}{2}$  to 5 mils in thickness and the other layer about 5 to 20 and preferably 8 to 12 mils. As previously indicated the preferred multilayered label is one of having a solid layer of polystyrene for treating with the solvent.

For some applications, the underside of an insoluble solid layer can be provided with, by printing, or some other suitable means a soluble, compatible solid polymer overlying the label layer in the areas to be formed into the finite areas.

Methylene chloride is a highly preferred solvent for use with the polystyrene foam. Methylene chloride, as set forth in the literature such as in the Solvents Chart in the 1968 Modern Plastics Encyclopedia, pg. 66, or in Plastics Engineering Handbook, 4th Edition, 1976 (Frados) or in Polymer Handbook, 2nd Edition, 1975 (Bandrup and Immergut); has a boiling point of about 39.8° C. and a solubility parameter of 9.7 (cal/cm<sup>3</sup>)<sup>1/2</sup>.

Generally, solvents having a solubility parameter of about 8.4 to 10.0 can be substituted for all or part of the methylene chloride.

Solvents for polystyrene that are suitable for use in the present invention include benzene, toluene, styrene, other lower chlorinated aliphatic hydrocarbons (such as trichloroethylene and perchloroethylene), methyl ethyl ketone and ethyl acetate.

Preferably, the boiling points of the solvents or suitable mixtures thereof are about 35° to 85° C. when the solvent is applied to the solid polystyrene layer at about room temperature (25° C.) or about 22° to 28° C.

Solvents suitable for use with polyvinyl chloride are benzene, toluene, ethylbenzene, styrene, and lower chlorinated aliphatic hydrocarbons including trichloroethylene and perchloroethylene. As in the case of polystyrene, methylene chloride is the preferred solvent.

Methylene chloride is the preferred solvent for the polyacrylates, other suitable solvents being those listed above for polyvinyl chloride.

Although not as preferred for polyvinylchloride and polyacrylates suitable solvents that can be used are methyl ethyl ketone, methyl formate, ethylene chloride and ethyl acetate.

As seen in the table headed "Solvents and Non-Solvents", Section IV, pages 241-265, and pages 349-359 of the previously mentioned Polymer Handbook; the solubility parameter for polyvinyl chloride generally is from about 9.4 to 10.8 (cal/cm<sup>3</sup>)<sup>1/2</sup> and for acrylate polymers and acrylic polymers is from about 8.2 to 11. As used in the above table, the solubility parameter of a polymer is defined at page IV-337 as the same as that of a solvent in which the polymer will mix (a) in all proportions, (b) without heat change, (c) without volume change, and (d) without reaction or special association.

The solvent used in the present invention can be a single solvent or a mixture of solvents. The solvent can be a solvent-polymer system in which the polymer is compatible with the label polymer. When the label polymer is polystyrene, a solvent-polymer system is one in which polystyrene has been dissolved in the solvent. A compatible polymer for polystyrene is a styrenic polymer as previously described.

Such solvent polymer systems as well as a single solvent or mixture of solvents, create the finite areas of the underside of the label by forming the momentary tacky solution of the polymer of the finite area in the solvent that allows the label to be tacked to the container for wrapping and also allows the label ends to be overlapped and stuck together to form the side seam.

I claim:

1. A container having a neck and a body, and a plastic label wrapped around the body, the label made of a thermoplastic polymer that is printable and is soluble in a solvent or a solvent polymer system compatible with the label polymer, the label comprising a solid polymer layer having a side that contacts the body and is attached lightly but securely thereto, the foam layer having a leading edge for contacting the body, there being a finite area on the leading edge having a liquid viscous solution of a polymer in a solution in the finite area being adapted to solidify and form a solid bond, the solution forming a momentary tacky bond sufficient to anchor the leading edges to the container body whereby the label can be wrapped around the body, the bond between the label and body becoming weaker as the solidifying solution hardens whereby the label can be easily removed from the container body for recycling without contaminating the material of the container body being reclaimed, the solid layer having a trailing edge that overlaps the leading edge to form a sleeve label with overlapped edges on the container body, and the solid layer of the trailing edge containing a second finite area generally extending along the trailing edge, the second finite area comprising a liquid tacky solution of a polymer in a solvent, the solution solidifying to form a side seam bond on the overlapped edges, the bond becoming stronger whereby, upon use, the side seam resists being pulled apart.

2. A container and label as defined in claim 1 in which the polymer of the finite areas is polystyrene and the solvent is methylene chloride.

3. A container and a label as defined in claim 1 in which the polymer of the finite areas is a styrenic poly-

mer comprising a copolymer of styrene and a copolymerizable vinyl monomer.

4. A container with a body portion and a plastic sleeve label wrapped around the body portion, the label comprising a solid thermoplastic printable polymer layer having an outer surface and an inner surface next to the body, the polymer layer being lightly but securely tacked to the body portion by a tacky adhesive bond formed from a finite area of the solid polymer, the finite area having a liquid tacky solution of the polymer in a quick evaporating low boiling point solvent for the polymer, the solution solidifying to form a solid adhesive bond after the label is wrapped, the bond between the finite area of the polymer layer and the container body becoming weaker as the tacky solution hardens whereby the label after use, can be easily removed from the container body to provide a clean container for recycling, the label having a seam formed by overlapping ends of the leading edge and the trailing edge of the label, the seam being bonded together by a liquid tacky solution of the polymer formed from the solid layer in a solvent therefor, the solvent being applied in a finite area along the trailing edge of the solid polymer layer to provide a liquid solution that solidifies to form the adhesive bond between the leading and trailing edges of the label at the label seam.

5. A coextruded plastic label having a solid polymer layer, there being a finite area along a first leading edge of the layer and a finite area along a second trailing edge of the layer, each of the finite areas having a liquid tacky solution of the polymer of the layer in a quickly evaporating solvent therefor, the solution solidifying to form a tacky adhesive bond in the finite area the solution of the finite area of the leading edge forming a momentary tacky bond sufficient to tack the label to a container for wrapping, the leading edge bond becoming weaker and weaker as the solvent rapidly cooperates.

6. A label as defined in claim 5 in which the polymer of the solid layer is polystyrene and the solvent is methylene chloride.

7. A label as defined in claim 5 in which there are a plurality of finite areas along the leading edge of the solid layer and the solvent has a solubility parameter of about 8.4 to 10.0 (cal/cm<sup>3</sup>)<sup>1/2</sup>.

8. A container and label as defined in claim 1 in which the container is an oriented polyethylene terephthalate container, the polymer of the solid layer is polystyrene, and the solvent is methylene chloride.

9. A container and label as defined in claim 1 in which the container is a glass container.

10. A container as defined in claim 1 in which the container is a metal container.

11. A container and label as defined in claim 1 in which the polymer of the finite areas is polyvinyl chloride.

12. A container and label as defined in claim 1 in which the polymer of the finite areas is an acrylate polymer.

13. A container having a neck and body, and a coextruded plastic label adapted for wrapping around the container body, the label comprising a thermoplastic, solvent-soluble, printable solid polymer layer having an outside surface with indicia thereon and an underside surface for attaching lightly but securely to the container body, the solid polymer layer having a leading edge for contacting the body, there being a finite area on the leading edge having a liquid viscous solution of

polymer from the solid polymer layer in a low boiling solvent for the polymer, the solution in the finite area being adapted to solidify and form an adhesive bond between the solidified polymer of the foam layer and the container body, the solution forming a momentary strong tacky bond sufficient to anchor the label to the body whereby the label can be wrapped around the body the bond between the finite area of the label and the body becoming weaker as the solidifying solution hardens whereby the label is easily removed from the container for clean recycling of the container, the solid layer having a trailing edge that overlaps the leading edge to form a tubular sleeve label with a side seam on the container body, the layer of the trailing edge having a finite area extending along said trailing edge in which

15

the finite area has a liquid tacky solution of the polymer of the finite area in a low boiling solvent, the solution solidifying to form a bond between the underside surface and the outside surface of the solid layer.

5 14. A container and label as defined in claim 1 in which the solvent has a boiling point of about 35° C. to 85° C. and a solubility parameter of about 8.4 to 10.0 (cal/cm<sup>3</sup>)<sup>1/2</sup>.

10 15. A container and label as defined in claim 13 in which the solvent has a solubility parameter of about 8.4 to 10.0 (cal/cm<sup>3</sup>)<sup>1/2</sup>.

16. A label as defined in claim 5 in which the solvent has a solubility parameter of about 8.4 to 10.0 (cal/cm<sup>3</sup>)<sup>1/2</sup>.

\* \* \* \* \*

20

25

30

35

40

45

50

55

60

65